

Aug. 7, 1923.

1,464,482

G. A. HENDERSON

## BITUMINOUS CONCRETE

Filed March 29, 1921

2 Sheets-Sheet 1



Inventor:  
George A. Anderson

Aug. 7 1923.

1,464,482

G. A. HENDERSON

BITUMINOUS CONCRETE

Filed March 29, 1921

2 Sheets-Sheet 2



Fig. 4.



Fig. 3.



Fig. 2.

Inventor:  
George A. Henderson

## UNITED STATES PATENT OFFICE.

GEORGE ASA HENDERSON, OF CHARLESTON, WEST VIRGINIA.

## BITUMINOUS CONCRETE.

Application filed March 29, 1921. Serial No. 456,563.

*To all whom it may concern:*

Be it known that I, GEORGE ASA HENDERSON, a citizen of the United States of America, residing at Charleston, in the 5 county of Kanawha and State of West Virginia, have invented new and useful Improvements in Bituminous Concrete, of which the following is a specification.

My invention relates to improvements 10 in plastic compositions in which pitch (of pétrolium or coal origin) or other plastic binder susceptible of becoming a fluid through the influence of applied heat, is used as the cementing agency of mineral or 15 vegetable aggregate, and particularly to products known as bituminous concrete, produced by the mixing method as distinguished from the so-called bituminous macadam produced by the penetration method 20 known to the trade.

The object of my invention is to produce increased density of such products heretofore produced from artificial asphalts or pitch as distinguished from the so-called 25 "natural" asphalts, such as that known to the trade as Trinidad Lake asphalt cement.

I have discovered that the product known 30 as natural Trinidad Lake asphalt, containing as it does approximately forty per cent mineral matter in the form of impalpable dust more or less colloidally suspended in its bitumen content, is the product of asphaltic base petroleum from which through 35 the agency of severe heat from volcanic eruption the lighter oils were volatilized during partial dehydration of the mass of asphaltic base petroleum, containing a clay deposit composed of mineral dust and water, by which natural operation the dust present 40 in the deposit at the time was, by the action of evolved steam, acting as a carrying agent, perfectly disseminated throughout the conglomerate in a state of colloidal dispersion. By tests of such natural pitch 45 as compared with tests of the so-called "arti-

ficial asphalts" such as that from asphaltic base petroleum from which the lighter oils are driven off, and entrap, by applied heat in refineries, I have discovered that the artificial product, or that produced by man 50 from such asphaltic base petroleum, as compared with that produced as aforesaid by nature from the identical character of base, viz, asphaltic base petroleum, is, at 77 degrees Fahr., of ductility over 60 cms., as 55 compared with the natural product (in the case of the Trinidad Lake product) of thirty eight (38) cms. at 77 degrees Fahr., that the proportion of bitumen soluble in 76 deg. Bé. naphtha in the case of the "artificial" product is 76.7%, while in the case 60 of the "natural" product that proportion of total bitumen thus soluble is 68.21% on an average of many tests, while on fluxing tests of 100 parts of each, the so-called 65 "Ohio residuum" in the case of the artificial product is nil as compared with 24 parts in the case of such "natural" asphalt; that the natural product as compared with the artificial product is more susceptible to 70 changes in temperature, is less ductile and cementitious and of a lower degree of purity, more affected by the action of water, and, as compared with 100 sq. yds. of 2" asphaltic concrete structures to 2000 lbs. of 75 the natural product, only 64 sq. yds. of 2" structure can be produced when using 2000 pounds of the so-called "natural" asphalt.

Accordingly I have discovered that while the bitumen content of the natural product 80 is inferior to that product of asphaltic base petroleum, containing 99.9% pure bitumen, in all essentials to paving structures, for example, nevertheless before the advent of the present invention, such paving structures produced of the natural asphalts containing said impalpable dust in colloidal suspension in extent approximately 40%, were and are superior to such products of the purer so-called "artificial asphalts," and 85

that this superiority is due solely to the combination of from 30% to 45% of impalpable dust content, so colloidally suspended in the structure, and to no other cause or agency, viz:

In the prior art of producing paving structures and the like from mineral and other aggregates mixed with a bituminous compound, any excess over ten per cent of 10 impalpable dust, (or that atomic matter that freely passes a 200 mesh sieve) is impracticable of agglomeration in any aggregate when mixed with a heavy bituminous binder (of approximately 50 penetration) 15 as distinguished from a light oily lubricant, (of approximately 100 penetration) and as a structure's inherent strength is measurable by that of its components bound together, impalpable dust in excess of such 20 ten per cent is prohibited in all United States and other standard specifications for bituminous concrete, (except those specifying the use of said Trinidad Lake asphalt) because it is known that no artificial means 25 have been provided for separating each dust particle from its neighbor, in such a structure, by a sufficiently thin film of such heavy bituminous binder (as distinguished from a light oily lubricant) to avoid an excess 30 of the binder itself in such structures.

In carrying out my process as described in my application Serial No. 212,194, filed Jan. 15, 1918, (Patent No. 1,370,815—Henderson) for Letters Patent of the United 35 States and elsewhere of sucking from the interstices between the larger aggregate, and from the surface of a worn macadam road, that dust thereof ground to impalpability by traffic and of incorporating that 40 dust by mixing it in air suspension with the heavier aggregate in a closure under suction and sufficient sustained heat, I have discovered that a considerable quantity of such dust is, by that means alone, entrapped 45 in the heavy mixing method bituminous compound, with each particle thereof surrounded by such binder; but I have discovered at the same time that a greater quantity of such dust can be so colloidally 50 interposed in a paving aggregate, in furtherance of the present object of this invention, by the additional means hereinafter described in combination with the above described step of the process, viz:

In my United States Patent No. 1,187,314, of 1916, (application Serial No. 874,934 filed Nov. 30, 1914) and improvements 55 thereof cited in my co-pending application now filed here in this Patent Office for fibrous compositions and process for making the same, I provide means for dehydrating a paving aggregate in the presence of molten bitumen, and in carrying out that process, in the manner described therein, I 60 have discovered that a considerable quantity

of impalpable dust in excess of said ten per cent can be, under the influence of suction and sustained heat sufficient to so dehydrate the entire mass, successfully incorporated in the final product in furtherance of the object here sought, of so using a substantial quantity, to-wit: in excess of 40% of such dust in a bituminous concrete structure.

I have further discovered that the combination of the above two essential steps of the present process results in its accomplishment of my object when the normally heavy (50 penetration) bituminous compound usually specified for bituminous concrete, or that produced by the so-called mixing method, is treated in the manner herein described, by which its fluidity is increased far beyond that possible by the mere agency of applied heat heretofore used exclusively for this purpose, provided such fluidity is of a temporary character, existing only during such mixing operation, without interfering with the consistency of a relatively hard nature of the bituminous compound, as tested for penetration, in the final product.

My invention will be best understood by reference to the accompanying drawing which will now be described, it being presumed, however, that various changes may be made in the apparatus by which the process is carried out without departing from the scope of the invention as defined in the appended claims.

Fig. 1 of the drawings is a view partly in side elevation and partly in vertical section of the apparatus adapted for carrying out the invention, and Fig. 2 is a cross sectional view of the apparatus taken on the line 2—2 of Fig. 1, showing the shafts and driving gears for the agitators in the hoppers and tank.

Fig. 3, is a sectional view, taken on line 3—3 of Fig. 1.

Fig. 4 is a sectional view, taken on line 4—4 of Fig. 1.

Supported on I-beams constituting the frame work of the machine, rests a bitumen storage tank N, braced internally with the members N<sup>1</sup>, N<sup>2</sup> also surrounding externally impregnating drum O rigidly anchored within the lines of tank N relatively near its bottom. Tank N is charged with bitumen preliminarily heated from an auxiliary supply thereof in heaters not shown, by the operation of pump N<sup>3</sup> forcing such heated bitumen into tank N thru inlet vent N'. In tank N this bitumen is maintained at the proper temperature, approximately 325 F., by means of steam pipes N<sup>4</sup> connected with boiler Q in which water is heated to produce the steam, by flues Q'. The steam from the boiler Q is conducted through pipe Q<sup>2</sup>, which pipe enters tank N just above the drum O

- and to the side of conveyor L' and extends and empties into manifold Q<sup>3</sup> connected with pipes N<sup>6</sup> and with manifold Q<sup>4</sup>, as shown. Surrounding drum O the heated bitumen tends to heat, indirectly, the contents of drum O, during the carrying out of the process. Bitumen outlet cock O<sup>9</sup> is manually opened, when tank N is to be emptied of its supply of bitumen, for any purpose.
- When approximately two-thirds full of the heated bitumen, the pump N<sup>a</sup> connection with the auxiliary supply is disconnected, and connected with influx suction pipe N<sup>a</sup>' the pump acting to lift the heated bitumen from the bottom of tank N on one side of drum O, and to move it up and through bitumen supply cock N A<sup>4</sup>, and down through pipe N<sup>a5</sup> to the reverse side of drum O in tank N at the top of the bitumen supply therein, thus providing a continuous agitation of the heating bitumen in tank N, and to afford ready access of the molten bitumen to the scale bucket E hereinafter described.
- Vegetable particles of the character denatured in accord with the process described in my United States Patent No. 1,187,314 for fibrous compositions and processes for making the same, are elevated by conveyor B to bins therefor provided, such as C. In the case of vegetable aggregate, the same is preliminarily dried to a residual moisture content of approximately 20%, that moisture residing at this stage of the process within the innermost pores of the vegetable particles. In the case of the mineral aggregate, the same shall contain atmospherically absorbed moisture, and in both cases the aggregate is so handled at this stage of the process, when it is of atmospheric temperature, and unheated otherwise.
- Mineral or other dust of impalpability is elevated via conveyor K to the bins R<sup>10</sup> and R<sup>11</sup> respectively, from a supply of such dust preliminarily provided at the base of the machine. This dust is of atmospheric temperature at this stage of the process, and may contain atmospherically absorbed moisture.
- Before placing the premelted bitumen in tank N the furnace QF' to boiler Q, preferably equipped with fuel oil burners, is operated by the lighting of the fuel supply, and motive power X, of any approved make or construction, shall operate to operate the moving members of the apparatus, viz: The revolution of driving shaft X' acts thru the cogs shown to revolve the drum O's central shaft O' suitably hung in proper bearings O<sup>7</sup> and O<sup>8</sup> as shown, and to revolve side longitudinal shaft X<sup>6</sup> in turn acting to operate thru pulley X<sup>7</sup>, belts X<sup>8</sup> and X<sup>8A</sup> exhauster X P thru pulley connection X<sup>9</sup>; pulley X<sup>10</sup>, with connection to pump driving pulley X<sup>11</sup>, cog X<sup>12</sup> with connection X<sup>13</sup> to pug mixers cog KJ<sup>2</sup>, acting to reciprocally operate cogs K<sup>1</sup>, K<sup>2</sup> and J<sup>1</sup> and J<sup>2</sup>, carrying interdigitating blades in the pug mixers K and J, designed to mix the ingredients thereto deposited in the manner hereinafter described; cog X<sup>14</sup>, revolving, by the connections shown, screw conveyor L', pulley and connections X<sup>15</sup> and X<sup>16</sup> to operate the revolving shaft, with agitating blades in dust and water mixer R' at pulley R'<sup>a</sup>, and to revolve gate valve R<sup>7</sup> from the bin R<sup>8</sup>, supplied with dust thru measuring scale bins R<sup>9a</sup> to be deposited, thru chute R<sup>6</sup>, in the manner hereinafter described.
- The operation of exhauster P acts in lieu of a stack to the furnace of boiler Q, to cause a draft of the hot air together with the products of combustion from said furnace, thru the flues of the furnace Q<sup>1</sup>, all emptying into dust chamber R, and thence thru the drum O from the point O<sup>3</sup> to the discharge chamber N<sup>7</sup> at the point O<sup>5</sup>, and out of the stack as shown.
- The exact temperature of the drum O, and its contents, is fixed by (a) the temperature of the bitumen in tank N, regulated by the relative degree of heat supplied to steam pipes N<sup>6</sup>, and (b) by the direct heat to said drum O's contents from the furnace, sucked therethru by the exhauster P. At the point marked R<sup>8</sup>, is provided an air inlet valve, manually operated, to cause an influx of air of atmospheric temperature from the outside, into dust chamber R, where, being mixed in the desired proportion with the hot air sucked thereinto from the furnace in the manner described, the temperature of the hot air to drum O is thus fixed at sufficient merely to raise the temperature of the mass in drum O at 250 deg. Fahr., as registered by approved thermometer stationed in the wall of the drum within sight of the operator.
- Two operators are proposed to be stationed on working platform V, one on either side of the pug mixers K and J, shown in the drawing. In charging the machine, which operates to discharge the material prepared in accord with this process, in a continuous flow thru discharge chamber N<sup>7</sup> at the screw conveyor O<sup>6</sup>, to the atmosphere, operator No. 1 opens cock N<sup>a4</sup> to discharge a pre-determined quantity of bituminous compound from tank N thru said cock into weigh bucket E equipped with scale beam, designed to travel on trolley D<sup>2</sup> by being manually pushed by the operator back and forth for the purpose of discharging, when the proper quantity of said bituminous compound has been measured thereinto, approximately one-half of said charge into pug mixer J and one half into pug mixer K. Simultaneously a predetermined quantity of the larger mineral or vegetable aggregate, or the two mixed together, containing residual

moisture and of atmospheric temperature, is by the manipulation of lever  $D^3$  deposited into weigh bin  $D$ , pivoted and hung by the member  $D'$  on trolley  $D^2$  in such a manner that the same may be, when the locking device, not shown, is released by the operator, tilted to discharge the contents of measuring bin  $D$  into pug mixer  $J$ , to be therein mixed by revolving interdigitating blades with the molten bitumen therein contained. Simultaneously operator No. 2 discharges, after measuring predetermined quantities of dust of impalpability, from bins  $R^{10}$  and  $R^{11}$  into weigh-bins, equipped with scale beams,  $R^8$ , approximately one-half of the designed proportion into mixer  $R'$  while simultaneously depositing therein water thru cock  $W$ , in quantity sufficient to produce a plastic composition of dust and water, which, being agitated sufficiently in mixer  $R'$  by the revolution of its shaft  $R^a$ , carrying agitating blades in the mixer, not shown, permeates and completely coats each atom of the dust with the water. The other half of the said dust charge is, simultaneously with the above operation deposited by operator No. 2 into chamber  $R^s$  from which chamber it is designed, by gravity, to fall into one of the four compartments of gate valve  $R^7$ , revolved at 20% of 1 R. P. M. to deposit within dust chute  $R^s$  one-half of the aforesaid dust charge within five minutes time. This dust is precipitated, gradually, by gravity, into dust chamber  $R$ , and is in said dust chamber constantly lifted by the spoon shaped agitating blades  $R^2$ , and dropped vertically therein, until all of that dust is, in air suspension, sucked in a heated condition, with the hot air and fumes from the furnace, directed into said dust chamber through the end of the boiler  $Q$  flues emptying thereinto, through said dust chamber and into drum  $O$  in a continuous flow, to be there entrapped by its adhering to the revolving blades  $O^2$  anchored to central shaft  $O'$  in drum  $O$ , and by the larger aggregate being therein manipulated in the manner hereinafter described.

In case there exists in the dust precipitated into chamber  $R$ , any particles too heavy or large to be carried in said air suspension to drum  $O$ , these are accumulated at the bottom of chamber  $R$ , from whence they are manually removed from time to time, by the instant opening and closing of sliding gate  $R^4$ , precipitating them to chamber  $R^s$  from which they are removed and discarded at the end of each day, or oftener if need be, manually.

The apparatus is designed to operate automatically to the extent of providing the proper proportion of the ingredients through the measuring devices above described, to the pug mixers, and otherwise, to provide for the continuous operation of the

various units of the apparatus reciprocally, as for example: The drum  $O$ , when of a fixed capacity of 1000 sq. yds. of  $1\frac{1}{2}$ " paving compacted in place per 8-hour day, of weight 100 pounds to the sq. yd. of finished product, is constructed of volume capacity to manipulate within five minutes and to discharge within that time through 12 feet of its length 1000 pounds of the material by the revolution of central shaft  $O'$ , carrying 36 agitating blades  $O^2$  of dimensions 6" at greatest (end) width tapering to 2" at the shaft-sleeve is fixed at 14 R. P. M., it being discovered by me that when set as shown in the drawing, these blades have a play each of 4" of the longitudinal length of said drum, and the material is moved by each blade 2" instead of four inches at each stroke, by reason of the tendency of approximately half of the material dropping vertically, and not being moved longitudinally more than 50% of the effective capacity of the blades' ends. When for example such material is mixed in the proportions, viz, containing in the final product in pounds and by per cent weight, sulfo-chlorinated bitumen 22, denatured wood particles 12.5, broken stone 52.2 and keiselguhr 13, (when the respective weights of said ingredients are as follows: Bituminous compound, per cu. ft. vol. cold, 70 lbs., keiselguhr per cu. ft., uncompacted, 15 lbs., dry wood fiber, uncompacted, uncontracted, per cu. ft. 10 lbs., and stone per cu. ft. of sizes 1" to  $1\frac{1}{4}$ ", 100 lbs.), 1000 pounds of the aggregate on the basis of the final product, with proper allowance being made for the initial moisture content at beginning of the operation, shall be weighed and manipulated through the aforesaid pug mixers, leading through screw conveyor  $L'$  to drum  $O$  in a continuous flow per five minutes of the plant's operation, viz:

The mixers  $K$  and  $J$  simultaneously mix for not exceeding one minute the proper proportions of the materials, deposited therein in the manner aforesaid. In mixer  $J$ , the residual moisture content of the aggregate reduces the temperature of the bitumen from approximately 325 to 250 deg. at which it is deposited in the mixer  $J$ , in combination with the cooling influence of the said aggregate of atmospheric temperature, to a degree that results in the temperature of the mixture, within one minute in said mixer  $J$  being approximately 175 deg. F., or under that temperature at which the moisture within the pores of the wood or of the stone becomes steam. However, in mixer  $K$ , where the dust mixed with water in the form of clay is deposited with 325 deg. Fahr. bitumen, in the proportions above given (with consideration given to the fact that but one-half of the proposed charge of dust passes thru this mixer, the

other half going to the dust chamber for manipulation in air suspension in the mass later) steam is evolved (which as per common knowledge is approximately 1600 times 5 the volume of the moisture from which it is evolved) with the result that in mixer K, the volume as deposited therein is increased, by ebullition, the steam acting as a carrying agent of the fine dust, to approximately ten 10 times that of the cold paste therein deposited. Whereupon, within the space of one minute, both mixers K and F, by manually opening of their bottoms thru the use of lever KJ', dump their contents simultaneously 15 by gravity to within chamber L, from which they are precipitated by gravity thru common open gate onto screw conveyor L' which operates to move from the chamber L its entire contents to the drum O, at the 20 point L<sup>2</sup> within the aforesaid five minutes, the shaft revolved by the cogged connection X-14 being fixed at the proper revolution per minute to accomplish this result. This operation being repeated through the 25 batch mixers, as described, every five minutes, there is provided a continuous flow of measured mixed material into drum O during the entire time of its operation.

The fumes and vapors from chamber L 30 are sucked out of that chamber and discharged to the atmosphere by the action of exhauster P acting thru outlet pipe L<sup>3</sup> as shown. The fumes and vapors from the bitumen storage and heating tank N, are 35 likewise removed therefrom by suction of exhauster P, by its action in connection with outlet pipe N<sup>5</sup> as shown.

It will be noted that the agitators O<sub>2</sub> are 40 designed to be so set on central shaft O' as to form a perfect screw, to move the material within drum O from its front to discharge chamber into which it drops by gravity onto cross screw conveyor O<sup>6</sup> stationed at its bottom, and revolved at fixed R. P. M. 45 by the machine's motive power, to discharge the mixed material either into trucks, not shown, for carting to the previously prepared road base, and thereon spread and compacted, or into molds for the manufacture 50 of the product in block form, or otherwise used as hereinafter specified.

The complete dehydration of the mixture is accomplished in the impregnating drum O, it being designed that when therein subjected 55 to the provided suction, shown, under the fixed degree of sufficient heat, sufficiently sustained, for the purpose, a thoroughly dry product, in the common acceptation of the term, is produced of initially wet material.

The fluidity, during mixing, of the bituminous compound, I produce in the following manner: (a) By mixing with the asphaltic product of asphaltic base petroleum or pitch, from 6 to 14% of sulfur, 65

and one-half of 1% of sulphate of copper, and relying on the partial volatilization of the oily constituent, under the influence of heat, to entrap the sulfur and its components within the bituminous compound, and then adding, to the sulfuretted bitumen in the impregnating drum, chlorine by injecting the same, in the form of chlorine gas, in measured quantities, thru dust chamber R, from a tube containing chlorine 70 therefor provided. I have discovered that the chlorine gas in passing thru the drum O marries to the sulfur in the bitumen therein contained, producing sulfur-chloride, and in combination with the bitumen, producing 75 sulfo-chlorinated-bitumen, which I have discovered produces, when mixed with mineral and vegetable aggregates for paving, flooring and such purposes, a product of greater cementing qualities, of greater ductility, and less affectable by atmospheric temperature changes, than any other such structure of which I have knowledge. Due to the fact 80 that it is the chemical action of the entrapped sulfur and chloride on the bituminous compound, affecting, in actually vulcanizing, the entire structure, that results in its ductility aforesaid, it is noteworthy 85 that this chemical agency is not volatilized and lost in time to the atmosphere as is the oily constituent of such bitumens heretofore relied on for continued life of the bituminous ingredient of paving, flooring, insulation, roofing and such products.

In a modified procedure in this regard, I take the fumes of heated sulfur and copper sulfate and pass them by said suction from their source, in the furnace proper, thru the dust chamber to the drum, and in the dust chamber I inject chlorine gas, which immediately marries with the sulfur product producing sulfur chloride, which in turn mixes, under the influence of such suction in the drum with the bitumen and aggregate while the same is being dehydrated, 100 producing hydrated sulfo-chlorinated bitumen, during the process of completely dehydrating the aggregate by the removal in the said drum, in the manner above described, of its residual moisture content, 105 under sufficient heat and suction, and I have discovered that this condition results in the temporary extreme fluidity of the heavy bituminous compound, only during dehydration thereof, required for its perfect agglomeration, entrapping in true colloidal suspension, the required substantial quantity of impalpable dust in the final product. The steam formed in said drum is sucked 110 out of it as well as out of the agitating material therein, completely by the aforesaid action of exhauster P, in the manner shown. In a modification of the invention in its relation to the final product produced 115 therefrom, I do not limit myself to the ex-

act apparatus as shown in the drawing illustrating the process, nor to the product of bituminous concrete in sheet and block form hereinabove described, but, after the material is prepared in the manner above described, it may be spread, from the machine of a portable nature as the machine is drawn, over the surface of a worn macadam road, for example, reliance on the machine itself being in this instance had to accomplish the following results: In lieu of the boiler and furnace described and shown in the drawing herewith, the furnace of the apparatus may consist of two steel sides supported on elliptical springs anchored between the sides and the bottom of bitumen storage tank N, the lower edges of which furnace sides scrape over the old roadway in course of its preparation to receive the new material hereinabove described. The front wheel of this machine is like unto that of a ten ton three wheel steam self-propelled road roller, and its tread is equipped with spikes, designed to break the old metal of the road. Immediately following this roller, and within the zone of the aforesaid two sides, (which act to retain in said "furnace" all supplied heat, without lateral suction of cold air from the outside) are provided tynes extending approximately 8 feet in width of the roadway under treatment, which act to scarify the broken road surface to a depth of approximately  $2\frac{1}{2}$ " thereof. Immediately following these tynes, I provide fuel oil burners, acting under compressed air, capable of throwing backward and down onto the road's surface approximately 1500 cu. ft. of hot air and flame mixed, per minute. This blast acts to blow out of the loosened interstices of the old road's stone, scarified, all dust and to heat the stone remaining on the road. This dust together with the products of the fuel oil combustion, is sucked up through two large flues, extending from the dust chamber R, shown in the drawing, through its bottom, to their opening over the roadway, the furnace above referred to being composed as follows: its bottom is the road's surface; its top is the bottom of the bitumen storage tank, and its sides are provided as hereinabove described. No part of the weight of the machine rests on the aforesaid sides, the rear of the machine being supported on two side wheels, and the front by the aforesaid roller wheel above described.

The dust thus removed from the interstices of the heated stone on the roadway, is sucked into drum O shown in the drawing after being mixed, in said dust chamber with the sulfur, additional dust added thru the chute R<sup>e</sup> by the operator, in measured quantity, as above described, and mixed

with the new aggregate prepared as in this specification described.

At the rear end of the aforesaid furnace is provided bitumen penetration nozzles, preferably of the rotary type, supplied with bitumen from an auxiliary supply in a tank on motor driven truck acting as a traction unit of the entire plant, and, under pressure, being conducted thru a supply pipe from said truck back through the top of said furnace to the aforesaid nozzles, manually operated by an operator stationed there, to deposit, and force within the dust cleared, loose heated stone of the roadway, an adequate quantity of preheated bitumen sufficient to coat said mineral aggregate on the road during turning of the same, by tynes placed within the radius of the effective nozzle spraying capacity. As the machine thus passes over the roadway, the new material emerges from the mouth O<sup>e</sup> of discharge chamber N<sup>e</sup>, is chuted to place, manually raked to a depth of approximately one inch, uncompacted, and steam roller compression is relied on to press the new hot material, at approximately 250 deg. Fahr., down and within the open interstices of the heated, bitumen-covered stone, in the absence of dust, until the larger stone remaining on the roadway shows on its surface a mosaic-like appearance.

In this manner I produce a 2" to  $2\frac{1}{2}$ " bituminous concrete wearing surface of mixed material, by the use of approximately 25% of new material added to the old, in approximate situ.

In cases where the width of the roadway is in excess of eight feet, two lateral sections are in the above manner constructed, a temporary steel curbing being spiked to the old surface in its center, and upon final rolling of the last section constructed, this curb is removed, and the space (about 4 inches) between the two sections, is filled with the new material, and rolling continued until no joint appears between the two.

It will be noted that the entire depth of approximately  $2\frac{1}{2}$ " of this structure is prepared while all of the ingredients forming it are hot, and that no dust is present to interfere with penetration of the bitumen thru the nozzles, into the open interstices of the road's stone during this part of the operation.

The above modification of the present process is to correct the conditions in this regard present in the prior art, viz: It is known that a light oily liquid (known as "road oil") will penetrate a cold road aggregate, and the dust on its surface, as well as that dust leached, in time, to and within the interstices of such an old road, by permeating it, as would a similar liquid such

as water; but that such a heavy bituminous binder as that standardized for the mixing method (as distinguished from such road oil, dust layer, or lubricant, both known to 5 the trade and prior art) will mat on the top of such a roadway, and not penetrate the interstices, or even bind the dust, but balls and rolls, if laid to any substantial thickness as such a mat, whereas the lighter oil 10 that will so penetrate the roadway is not a binder in the true sense as used in bituminous concrete or the "mixing method" for producing paving structures, and merely acts as a lubricant, or temporary dust-layer 15 to be renewed annually, to form a built-up structure of inferior-lasting quality to that herein proposed.

I claim:

1. The process of manufacturing a bitumi- 20 nous composition, consisting in preheating, while agitating, a relatively hard bituminous cement to a temperature of approximately 325 deg. Fahr.; then preparing by wetting and comminuting a fibrous vegetable ag- 25 gregate and then removing therefrom a por- 30 tion of its water content; then depositing the fibrous material, when at atmospheric temperature and containing its residual moisture into a mixer equipped with re- 35 volving interdigitating blades containing the heated bitumen during agitation of the mass therein to reduce the temperature of the bitumen and of the mass to approxi- 40 mately 175 deg. Fahr.; then subjecting the 45 mass during continued agitation thereof, to sufficient heat, sufficiently sustained for the purpose of raising the temperature of the mass to a degree above the boiling point of water, to cause ebullition of the mass by the 50 creation therein of steam from the residual moisture, to act as a carrying agent of the ingredients, and to separate the fibers from each other during said agitation of the mass, and continuing the operation under sus- 55 tained heat sufficient to produce a thor- 60oughly dry product from the initially wet material; then compacting the same in molds to shape, substantially as described.

2. The process of producing a bituminous 50 conglomerate, the inherent density of which is characterized by colloidal dispersion of mineral dust and vegetable fibers uniformly throughout its mass, consisting in depositing comminuted fibrous vegetable material 55 containing in excess of 20% moisture and truly colloidal keiselguhr, (an impalpable silica so finely divided as to form atomic matter all of which freely passes a 200 mesh sieve) at atmospheric temperature in a mixer 60 equipped with revolving interdigitating blades, containing a predetermined proportion of bitumen preheated to a temperature above 325 deg. Fahr., and subjecting the 65 mass therein to sufficient heat sufficiently sustained, during continuous agitation of the

mass, to colloidally disperse the fibers and mineral dust throughout the bitumen during complete dehydration of the mass; then removing the mass from the mixer while hot and compacting the same in molds to shape, substantially as described. 70

3. The process of producing a fibrous composition for insulation, roofing, paving and other purposes, consisting in introducing into a mixer to preheated bitumen, moist fibrous material and truly colloidal dust, all passing a 200 mesh sieve, at atmospheric temperature, in proportions of each predetermined and mechanically fixed by measuring devices at the mixer; then subjecting the mass to sufficient heat, sufficiently sustained, to cause ebullition of the mass during continuous kneading of the same by revolving interdigitating blades until, during the process of complete dehydration of the mass, the fibrous material and filler-dust are in a state of colloidal, dispersion within the bitumen constituting the continuous phase of a thoroughly dry product of initially wet material, substantially as described. 80 85 90

4. The process of producing a dense bituminous composition consisting in reducing a relatively hard bituminous cement to fluidity by heat in the presence of steam acting as its carrying agent while separating, during mechanical agitation of, moist vegetable fibers in the presence of the bitumen in a mixer equipped with revolving interdigitating blades; then cooling the mass to a temperature below the boiling point of water; then reheating the mass in said mixer, subjecting it to sustained heat sufficient in degree and duration to raise the temperature of the mass to approximately 250 deg. Fahr., during dehydration of the mass required for its perfect agglomeration and entrapping in truly colloidal suspension of from 20 to 45 % of added impalpable dust in sizes that all of the particles thereof shall pass a 200 mesh sieve, in the final product by the process of forming steam of the residual moisture in the agitated material; then compressing the mass to shape in molds, substantially as described. 100 105 110

5. The process of producing a bituminous concrete consisting in preliminarily wetting colloidal mineral dust, all of which freely passes a 200 mesh sieve, and vegetable fibrous material, removing their excess water content, and the completely dehydrating the aggregate in the presence of a relatively hard bituminous compound temporarily reduced to fluidity by heat while subjecting the mass to sustained heat sufficient in degree and duration to completely dehydrate the mass during agitation of the same in a batch mixer operating to distribute the aggregate throughout, the bitumen acting as the continuous phase of the conglomerate while separating the fibers and dust therein 115 120 125 130

in a state of colloidal dispersion, then tilting the mixer to discharge its contents into molds, and then compacting the same there-in to shape substantially as described.

5. 6. A bituminous fibrous composition consisting of hard bituminous cement, fibrous material and in excess of 40% mineral dust all particles of which are sufficiently divided to freely pass a 200 mesh sieve, colloidally suspended in the relatively hard bituminous cement which has a ductility over 60 cms. at 77 deg. Fahr., acting as the impregnating, coating and binding agent of and as the continuous phase in colloidal dispersion of the 10 separated fibers which reinforces the mass.

7. A bituminous conglomerate of vegetable fibers impregnated with a relatively hard bitumen of ductility exceeding 60 cms. at 77 deg. Fahr., and colloidally suspending keiselguhr in particles all passing a 200 mesh sieve, and acting as the continuous phase in colloidal dispersion of the vegetable fibers.

In witness whereof I have hereunto set my hand in the presence of two witnesses this 25 sixteenth day of October, 1920.

GEORGE ASA HENDERSON.

Witnesses:

J. H. DUNLAP,  
W. A. BURGESS.